

## UNITED STATES PATENT OFFICE

2,227,952

## SULPHURIZED OIL

John C. Zimmer, Hillside, N. J., assignor to Standard Oil Development Company, a corporation of Delaware

No Drawing. Application July 20, 1938,  
Serial No. 220,267

17 Claims. (Cl. 252—46)

The present invention relates to improved sulphochlorinated oils and to methods for making the same. The invention will be fully understood from the following description:

5 It has been known for many years that sulphur and chlorine increased the load bearing capacity of oils for lubrication of hypoid and other gears where high or extreme pressures may be encountered, metal working and the like and many such oils have been and are now used for these purposes. In some cases mineral oils have been sulphurized directly; in others fatty oils such as lard and fish oils are sulphurized and are added to the mineral bases. Both of these products serve the purpose but at the same time have many disadvantages; for example, it is difficult to add enough sulphur to mineral oils to give sufficient load bearing capacity, without encountering sulphur separation when the product is cooled. Sulphurized fatty oils containing more than 10 to 12% of sulphur have a very foul odor which is objectionable in cutting oils and the like, and if the sulphur content is reduced the extreme pressure properties are greatly impaired.

10 Moreover, their blends in mineral oil do not possess sufficient extreme pressure properties for satisfactory lubrication of automotive hypoid gears, and the sulphurized fatty oil is often not completely soluble in mineral oil and tends to separate in storage and service.

Similar difficulties occur with the various other sulphurized bases which have been suggested from time to time.

It has now been found that these difficulties can be overcome by using as the base to be sulphurized a solvent extraction product of petroleum. The extract is obtained by the use of solvents such as phenol, cresol, dichlor ethyl ether, aniline, sulphur dioxide, nitro benzol, furfural, and the like, which various solvents with others, too numerous to specifically mention, make up the class of extraction solvents which are used to separate liquid paraffinic constituents from non-paraffinic fractions. The extracts may be obtained from petroleum fractions such as kerosene, gas oils, and the light and heavy lubricating fractions. The quality of the extract depends of course to some extent upon the crude from which it is obtained and the intensity of the extraction treatment, but for present purposes it has been found that an extract having a viscosity index below about +50 is suitable for the purpose, although it is preferred to use materials having a lower viscosity index, for example below 0, -5 or -10, or even lower. The

extracts may be obtained from paraffinic, naphthenic, or mixed asphaltic base type of crude oils. In general the preferred stocks are those rich in natural sulphur, for example, the original sulphur content varies from say 0.6 to 3 or 4% of the extract.

15 The extract is preferably purified first by treatment with sulphuric acid in the same way that most mineral oils are refined. This removes the more unstable asphaltic products and gives a much more desirable stock to sulphurize. Ordinarily from 5 to 15 pounds of acid per barrel are used in the preliminary treatment.

The mineral oil extract is sulphurized by treatment with a suitable sulphur halide among which sulphur monochloride is the most suitable. The extract sulphurizes much more readily than an ordinary mineral oil, in fact so readily that great care should be taken to prevent too vigorous action which tends to formation of insoluble, sludge-like products. This is best accomplished by limiting the amount of sulphur chloride used to approximately 5 to 15% of the extract. With amounts up to 5% of the extract there is little or no sludge and more may be used but there is an increasing tendency to sludge. This is offset to some degree by the first step of sulphuric acid refining, but for most purposes effective compounds which are stable and possess good extreme pressure qualities may be made with approximately 5% of sulphur chloride. Broadly, however, a greater range of sulphur chloride is useful, for example up to 20 or 25%. The temperature of treatment is from about 100° F. to 35 about 300° F. and, as stated before, the reaction is rapid and vigorous, much more so than is usually the case with mineral oil.

40 It has been found that the extraction products referred to above may be used alone as the sulphochlorinated stock, or it may be used to replace a certain amount of the fatty oil which has previously been employed. In some instances, it is desirable to have some of the fatty oil present and in these cases the extraction product and the fatty oil may either be sulphurized separately and mixed or may be admixed and sulphurized together, for example, in proportion of say 10 to 75% of the extraction product and 90 to 25% of fatty oil such as sperm oil, lard oil, rapeseed oil, or the like. The presence of the extraction product appears to greatly increase the ease of sulphurization and to improve the product obtained, particularly from 45 50 55

the standpoint of freedom from obnoxious odor and improved load carrying capacity.

The sulphochlorinated stock and the mineral lubricating oil containing the same may be used for many purposes. They may be employed in cutting oils or in oils used for other processes of metal working such as stamping, drawing and the like, wherever, in fact, sulphurized or sulphochlorinated oils are now employed, and the degree of sulphurization of the base and the amount of the base in the mineral oil may vary considerably depending on the particular use to which the oil is to be placed. Ordinarily the oil should contain from about 0.40% to 1.50% Cl and 2.5% to 4.0% S. The stock may also be used for gear lubrication, especially for the lubrication of steel gears operating under high pressures, for example in the automotive differentials or other gear units employing hypoid or other types of gears. For these purposes it is frequently desirable to add to the oil a soluble lead compound such as lead naphthenate or lead sulphonate, or their equivalents. Zinc soaps or mixture of zinc and lead soaps may be employed with advantage. Such materials should be added after the sulphurized stock has been cooled so as to prevent immediate reaction of the sulphur or chlorine with the lead, it being desired to obtain the materials in separate compounds in the final oil which is free from suspended solids.

The oils described and produced as above have excellent extreme pressure qualities which are not rapidly lost during the normal use of the oil which is one of the chief objections to many of the products now available. These oils show no separation of solids and the viscosity index of the finished blend is not so greatly reduced by the use of a sulphurized extract as would be supposed. For example, where an unsulphurized extract is added to a mineral oil of 95 to 100 V. I. in quantity sufficient to give a reduction in viscosity index from 70 to 75, it has been found that after sulphurization, the same amount of the extract produced a blend of from 85 to 90 V. I. In addition, the compounds are extremely stable during use even when subjected to oxidation. Many of the oils used at the present time oxidize so rapidly as to become solid after a few hours of severe oxidation or in severe high temperature gear service. These oils, however, have been found to thicken only slightly during such treatment.

In order to further illustrate the nature of the present products and the methods by which they are made, the following examples are offered:

#### Example I

A solvent extract of a light petroleum lubricating oil obtained by treatment with phenol had the following characteristics:

|                            |        |
|----------------------------|--------|
| Gravity, A. P. I.          | 15.1°  |
| Flash                      | 380    |
| Vis. @ 100° F.             | 591.8  |
| Vis. @ 210° F.             | 55.0   |
| V. I.                      | +2     |
| Pour point                 | -5° F. |
| Per cent sulphur (natural) | 0.98   |

This material was treated with 10 pounds of sulphuric acid to the barrel of oil, after which two separate samples were treated with 5 and 7.5% respectively of sulphur monochloride. Temperature was maintained at 240 to 260° F. during the treatment which required 2 hours.

The products were cooled and gave the following analyses:

|                             | No. 1   | No. 2 | 5     |
|-----------------------------|---------|-------|-------|
| Acid treated phenol extract | percent | 95    | 72.5  |
| Sulphur monochloride        | do      | 5     | 7.5   |
| Gravity                     |         | 15.1  | 13.1  |
| Vis. @ 100° F. Say. sec.    |         | 1,080 | 1,383 |
| Vis. @ 210° F.              | do      | 69    | 75    |
| Sediment                    | percent | 0.10  | 1.14  |
| Sulphur                     | do      | 3.27  | 3.78  |
| Chlorine                    | do      | .72   | 1.14  |

Of these two materials the one made with 5% S<sub>2</sub>Cl<sub>2</sub> is superior because of the low sediment. Both, however, were endowed with excellent extreme pressure properties as will be seen from the fact that the oils carried 15 weights in the Almen test when normally applied and also when applied rapidly under shock load conditions which are much more severe.

15

#### Example II

The two products prepared as in Example I were blended with equal volumes of mineral lubricating oils, and the inspections of the mineral oil used and of the two blends are as follows:

|                   | Mineral oil | Mineral oil blend 50% No. 1 | Mineral oil blend 50% No. 2 | 30   |
|-------------------|-------------|-----------------------------|-----------------------------|------|
| Gravity, A. P. I. | degrees     | 26.1                        |                             |      |
| Flash             | seconds     | 420                         |                             |      |
| Vis. @ 100° F.    | seconds     | 310                         | 666                         | 583  |
| Vis. @ 210° F.    | do          | 51                          | 61.2                        | 58.7 |
| V. I.             |             | 79                          | 42                          | 45   |
| Sulphur           | percent     | 0.25                        | 1.63                        | 1.89 |
| Chlorine          | do          |                             | 0.36                        | 0.57 |
| Sediment          | do          |                             | 0.03                        | 0.40 |

These blends were subjected to the Almen test with the result that again both carried the full 15 weights when normally applied and when applied under shock conditions.

40

#### Example III

A solvent extract of a light petroleum lubricating oil obtained by treatment with phenol and having the characteristics enumerated in Example I was mixed with an equal volume of No. 1 grade lard oil and then treated with 5% sulphur monochloride. Temperature was maintained at 250° to 260° F. for 2 hours. The product analyzed as follows:

|                           |          |       |
|---------------------------|----------|-------|
| Sulphur                   | per cent | 4.39  |
| Chlorine                  | per cent | 2.97  |
| Say. Univ. vis. @ 210° F. | sec      | 191.7 |

A blend of 10% of the above in a pale paraffin oil carried 15 weights on the Almen test under shock loading conditions.

55

#### Example IV

To the blend of sulphur-chloride treated oil last referred to in the previous example, 10% of lead naphthenate is added. This product was an excellent leaded oil for use in lubricant of hypoid gears or other severe service. This product carried the full 15 weights on the Almen test when applied under shock loading conditions.

60

The present invention is not to be limited by any theory of the mechanism of the present sulphurization process nor to the use of any particular ingredients, but only to the following claims in which it is desired to claim all novelty inherent in the invention.

65

I claim:

1. Process for producing an improved sulphur-chlorinated oil comprising reacting a substan-

70

75

- tially non-asphaltic solvent extraction product of a petroleum lubricating oil having a viscosity index below 50 at a temperature between 100 and 300° F. with 5 to 15% of sulphur monochloride until the product contains at least about 0.4% chlorine.
2. An improved process for preparing sulphur-chlorinated oil to resist high pressures which comprises blending a substantially non-asphaltic phenol extract of a petroleum lubricating oil with a fatty oil, then reacting the blend with 5 to 25% of sulphur chloride at a temperature of 150 to 300° F.
3. Process according to claim 2 in which 10 to 15 75% of the extraction product of petroleum is blended with 90 to 25% of a fatty oil and this mixture is subjected to the sulphurization.
4. A process for producing an improved sulphur-halogenated oil comprising reacting a substantially non-asphaltic solvent extract of a petroleum oil fraction at least as heavy as kerosene with a sulphur halide in an amount between about 5% and 25% at a temperature between about 100° and 300° F.
5. Process according to claim 4 in which the extract has a viscosity index below about 50 and is obtained from a petroleum lubricating oil which has been acid treated.
6. Process according to claim 4 in which said sulphur halide is a sulphur chloride.
7. Process according to claim 4 in which said sulphur halide is sulphur monochloride.
8. A process for producing an improved sulphur-chlorinated oil comprising reacting a substantially non-asphaltic phenol extract of a petroleum oil fraction at least as heavy as kerosene with a sulphur chloride in an amount between about 5% and 25% at a temperature between about 100° and 300° F.
9. A process for producing an improved sulphur-chlorinated oil comprising reacting a substantially non-asphaltic phenol extract of a petroleum lubricating oil fraction, said phenol extract having a viscosity index below 50, with a sulphur chloride in an amount between about 5% and 15% at a temperature between about 100° and 300° F.
10. A composition of matter comprising a sulphur-halogenated oil suitable for use in metal working processes for extreme pressure lubrication, said sulphur-halogenated oil being prepared by subjecting a substantially non-asphaltic solvent extract of a petroleum oil fraction at least as heavy as kerosene to reaction with a sulphur halide in an amount between about 5% and 25% at a temperature between about 100° and 300° F. with 5
11. A composition as described in claim 10 in which said sulphur halide is a sulphur chloride.
12. A composition as described in claim 10 in which said sulphur halide is sulphur monochloride.
13. A composition of matter comprising a sulphur-chlorinated oil suitable for use in metal working processes for extreme pressure lubrication, said sulphur-chlorinated oil being prepared by subjecting a phenol extract of a petroleum lubricating oil fraction, said phenol extract having a viscosity index below 50, to reaction with a sulphur chloride in an amount between about 5% and 25% at a temperature between about 100° and 300° F., the resulting sulphur-chlorinated oil containing from about 0.4% to 1.5% chlorine and from 2.5% to 4% sulphur.
14. A composition of matter comprising a sulphur-chlorinated oil suitable for use in metal working processes for extreme pressure lubrication, said sulphur-chlorinated oil being prepared by subjecting a blend of about 90% to 25% of a fatty oil and 10% to 75% of a solvent extract of a substantially non-asphaltic solvent extract of a petroleum oil fraction at least as heavy as kerosene, to reaction with sulphur chloride in an amount between about 5% and 25% at a temperature between about 100° and 300° F.
15. An improved sulphur-and-halogen-compounded oil suitable for use in metal working processes for extreme pressure lubrication comprising a blend of a lubricating oil and the sulphur-halogenated oil described in claim 10.
16. An improved sulphur-and-chlorine-compounded oil suitable for use in metal working processes for extreme pressure lubrication comprising 70 to 95 parts of a mineral lubricating oil and 30 to 5 parts of the sulphur-chlorinated oil described in claim 13.
17. An improved sulphur-and-chlorine-compounded oil suitable for use in metal working processes for extreme pressure lubrication comprising 70 to 95 parts of a petroleum lubricating oil having a viscosity index above 80 and 30 to 5 parts of the sulphur-chlorinated oil described in claim 13.

JOHN C. ZIMMER.